

## UNITED STATES PATENT OFFICE.

CLARENCE I. B. HENNING, OF WILMINGTON, DELAWARE, ASSIGNOR TO E. I. DU PONT DE NEMOURS & COMPANY, OF WILMINGTON, DELAWARE, A CORPORATION OF DELAWARE.

## IGNITING MIXTURE.

No Drawing.

Application filed November 17, 1920. Serial No. 424,691.

*To all whom it may concern:*

Be it known that I, CLARENCE I. B. HENNING, a citizen of the United States, and a resident of Wilmington, in the county of New Castle and State of Delaware, have invented 5 a certain new and useful Igniting Mixture, of which the following is a specification.

This invention relates to priming mixtures for propellant explosives, and comprises a priming charge containing as an essential constituent tetrinitropentaerythrite.

In priming mixtures containing, for example, lead sulphocyanide, an oxidizing salt having a high oxygen content such as potassium chlorate, and trinitrotoluene, it has been found that if the amount of the last-mentioned substance be increased beyond 7%, the violence of the combustion of the mixture frequently drives the metal part of 20 the primer from the head of the shell.

It has been proposed to substitute tetrani- 25 tromethylaniline for the trinitrotoluene in priming mixtures of the kind described above, but these proposed primers are more brisant than those containing trinitrotoluene and have been found somewhat objectionable on this account. What is desired is a sus- 30 tained flame rather than a severe blow.

According to my invention tetrinitropentaerythrite is used in place of trinitrotoluene in primers of the above type. Tetrinitropentaerythrite has notable advantages in 35 that it is much less sensitive to friction or percussion than any of the compounds mentioned above; as a result the proportion thereof in the priming mixture can be increased without making the mixture too brisant. Tetrinitropentaerythrite has the further advantage of being little affected in 40 its rate of burning by changes in temperature; hence primers containing this ingredient burn uniformly and are less affected by changes in temperature than many other primers now in use.

Priming compositions made in accordance 45 with my invention may be illustrated by the following examples:—

The proportions of the several ingredi- 55 ents of the priming mixtures may vary considerably; the proportion of tetrinitropentaerythrite present should preferably be from about 5 to 10% of the total mixture.

In connection with the use of modern pro- 60 gressive burning smokeless powders, it is desirable to have a priming mixture which will give the maximum energy and igniting power. The chemical and physical properties of tetrinitropentaerythrite are such that 65 the increase in energy, heat and flame delivered per unit of weight will be much greater than that given by any substance heretofore used in priming compositions.

Priming mixtures of the kind above de- 70 scribed are extensively used in connection with small arms ammunition.

I claim:

1. An igniting mixture for small arms ammunition containing tetrinitropentaerythrite, said mixture becoming ignited but not detonating when struck lightly, and being adapted to ignite a propellant explosive. 75

2. An igniting mixture comprising potassium chlorate, antimony sulphide, and tetrinitropentaerythrite. 80

3. An igniting mixture comprising potassium chlorate, antimony sulphide, and from about 5 to 10% of tetrinitropentaerythrite. 85

4. An igniting mixture comprising potassium chlorate, antimony sulphide, lead sulphocyanide, and tetrinitropentaerythrite. 90

5. An igniting mixture comprising 50 parts of potassium chlorate, from about 20 to 17 parts of antimony sulphide, from about 25 to 23 parts of lead sulphocyanide, and from about 5 to 10 parts of tetrinitropentaerythrite. 95

6. An igniting mixture comprising tetrinitropentaerythrite and an oxidizing salt having a high oxygen content. 95

In testimony whereof I affix my signature.

CLARENCE I. B. HENNING.

|                               | Parts by weight. |     |         |
|-------------------------------|------------------|-----|---------|
|                               | I.               | II. | III.    |
| Potassium chlorate.....       | 50               | 50  | 35      |
| Lead sulphocyanide.....       | 23               | 23  | —       |
| Antimony sulphide.....        | 20               | 17  | 30      |
| Tetrinitropentaerythrite..... | 5                | 10  | 5 to 10 |
| Mercury fulminate.....        | —                | —   | 35      |